



US005827635A

**United States Patent** [19]**Cole****Patent Number:** **5,827,635****Date of Patent:** **Oct. 27, 1998**

[54] **HIGH TEMPERATURE COLOR DEVELOPMENT OF PHOTOGRAPHIC SILVER BROMOIODIDE COLOR NEGATIVE FILMS USING STABILIZED COLOR DEVELOPER SOLUTION**

[75] Inventor: **David Leroy Cole**, Rochester, N.Y.

[73] Assignee: **Eastman Kodak Company**, Rochester, N.Y.

[21] Appl. No.: **916,559**

[22] Filed: **Aug. 22, 1997**

**Related U.S. Application Data**

[60] Division of Ser. No. 703,593, Aug. 27, 1996, abandoned, which is a continuation-in-part of Ser. No. 590,241, Jan. 23, 1996, abandoned.

[51] **Int. Cl.<sup>6</sup>** ..... **G03C 7/407**

[52] **U.S. Cl.** ..... **430/372; 430/434; 430/486; 430/490**

[58] **Field of Search** ..... **430/372, 434, 430/486, 490**

**[56] References Cited****U.S. PATENT DOCUMENTS**

|           |         |                 |         |
|-----------|---------|-----------------|---------|
| 4,629,683 | 12/1986 | Itoh et al.     | 430/390 |
| 4,798,783 | 1/1989  | Ishikawa et al. | 430/372 |
| 4,800,153 | 1/1989  | Morimoto et al. | 430/380 |
| 4,801,516 | 1/1989  | Ishikawa et al. | 430/380 |
| 4,814,260 | 3/1989  | Koboshi et al.  | 430/464 |
| 4,833,068 | 5/1989  | Ohki et al.     | 430/484 |
| 4,842,993 | 6/1989  | Yagihara et al. | 430/380 |
| 4,851,325 | 7/1989  | Morimoto et al. | 430/372 |
| 4,853,318 | 8/1989  | Fujita et al.   | 430/380 |
| 4,876,174 | 10/1989 | Ishikawa et al. | 430/380 |
| 4,892,804 | 1/1990  | Vincent et al.  | 430/380 |
| 4,897,339 | 1/1990  | Andoh et al.    | 430/372 |
| 4,956,267 | 9/1990  | Ueda et al.     | 430/372 |
| 4,963,475 | 10/1990 | Murai et al.    | 430/467 |
| 4,965,176 | 10/1990 | Ishikawa        | 430/378 |
| 4,966,834 | 10/1990 | Ishikawa et al. | 430/393 |
| 4,985,347 | 1/1991  | Fujimoto et al. | 430/393 |
| 5,028,517 | 7/1991  | Kuse et al.     | 430/434 |
| 5,053,322 | 10/1991 | Shiba et al.    | 430/464 |
| 5,066,571 | 11/1991 | Yoshida et al.  | 430/489 |
| 5,071,734 | 12/1991 | Ueda et al.     | 430/372 |
| 5,077,180 | 12/1991 | Yoshida et al.  | 430/380 |
| 5,091,292 | 2/1992  | Fujimoto et al. | 430/467 |
| 5,093,226 | 3/1992  | Ohshima         | 430/377 |
| 5,094,937 | 3/1992  | Morimoto        | 430/485 |
| 5,100,765 | 3/1992  | Fujimoto        | 430/434 |
| 5,110,713 | 5/1992  | Yoshida et al.  | 430/372 |
| 5,110,985 | 5/1992  | Hayakawa et al. | 562/571 |
| 5,128,237 | 7/1992  | Kimura et al.   | 430/378 |
| 5,147,766 | 9/1992  | Ishikawa et al. | 430/399 |
| 5,153,108 | 10/1992 | Ishikawa et al. | 430/376 |
| 5,153,111 | 10/1992 | Yoshida et al.  | 430/444 |
| 5,173,394 | 12/1992 | Hayashi         | 430/372 |
| 5,173,395 | 12/1992 | Asami           | 430/376 |
| 5,178,992 | 1/1993  | Yoshida et al.  | 430/372 |
| 5,202,229 | 4/1993  | Kuse et al.     | 430/399 |
| 5,204,229 | 4/1993  | Nakamura et al. | 430/399 |
| 5,230,991 | 7/1993  | Nagaoka et al.  | 430/393 |
| 5,236,814 | 8/1993  | Kuse et al.     | 430/393 |
| 5,238,789 | 8/1993  | Ohshima         | 430/372 |
| 5,246,819 | 9/1993  | Yoshida et al.  | 430/386 |

|           |         |                    |         |
|-----------|---------|--------------------|---------|
| 5,248,811 | 9/1993  | Morimoto           | 562/102 |
| 5,250,396 | 10/1993 | Ueda et al.        | 562/357 |
| 5,252,439 | 10/1993 | Nakamura           | 430/399 |
| 5,260,185 | 11/1993 | Takabayashi et al. | 430/491 |
| 5,262,563 | 11/1993 | Morimoto           | 430/104 |
| 5,344,750 | 9/1994  | Fujimoto et al.    | 430/434 |
| 5,354,646 | 10/1994 | Kobayashi et al.   | 430/372 |
| 5,362,610 | 11/1994 | Yoshimoto          | 430/465 |
| 5,376,509 | 12/1994 | Yoshimoto et al.   | 430/449 |

**FOREIGN PATENT DOCUMENTS**

|        |         |                    |   |
|--------|---------|--------------------|---|
| 269227 | 6/1988  | European Pat. Off. | . |
| 434097 | 6/1991  | European Pat. Off. | . |
| 468781 | 1/1992  | European Pat. Off. | . |
| 488217 | 6/1992  | European Pat. Off. | . |
| 488737 | 6/1992  | European Pat. Off. | . |
| 530921 | 3/1993  | European Pat. Off. | . |
| 540296 | 5/1993  | European Pat. Off. | . |
| 556782 | 8/1993  | European Pat. Off. | . |
| 574829 | 12/1993 | European Pat. Off. | . |
| 611986 | 8/1994  | European Pat. Off. | . |

**OTHER PUBLICATIONS**

|              |                  |
|--------------|------------------|
| JP 02-001846 | (Abstract only). |
| JP 02-018556 | (Abstract only). |
| JP 02-018557 | (Abstract only). |
| JP 03-075745 | (Abstract only). |
| JP 03-102344 | (Abstract only). |
| JP 03-127058 | (Abstract only). |
| JP 03-158849 | (Abstract only). |
| JP 03-184044 | (Abstract only). |
| JP 03-211547 | (Abstract only). |
| JP 03-259145 | (Abstract only). |
| JP 03-266837 | (Abstract only). |
| JP 04-063342 | (Abstract only). |
| JP 04-097355 | (Abstract only). |
| JP 63-32548  | (Abstract only). |
| JP 63-32549  | (Abstract only). |
| JP 63-40149  | (Abstract only). |
| JP 63-92949  | (Abstract only). |
| JP 63-264751 | (Abstract only). |
| JP 63-53551  | (Abstract only). |
| JP 63-48548  | (Abstract only). |
| JP 63-179351 | (Abstract only). |
| JP 63-306444 | (Abstract only). |
| JP 63-318557 | (Abstract only). |
| JP 01-124851 | (Abstract only). |
| JP 63-264752 | (Abstract only). |
| JP 01-187548 | (Abstract only). |
| JP 01-265250 | (Abstract only). |
| JP 04-340961 | (Abstract only). |
| JP 05-040333 | (Abstract only). |
| JP 04-366949 | (Abstract only). |

*Primary Examiner—Hoa Van Le  
Attorney, Agent, or Firm—J. Lanny Tucker*

[57]

**ABSTRACT**

Silver bromoiodide color negative films can be rapidly color developed using heat stabilized color developing solutions kept at high temperatures with minimal changes in the resulting color record densities. These advantages are achieved using specific hydroxylamine derivatives as antioxidants in the color developer solution.

**HIGH TEMPERATURE COLOR  
DEVELOPMENT OF PHOTOGRAPHIC  
SILVER BROMOIODIDE COLOR NEGATIVE  
FILMS USING STABILIZED COLOR  
DEVELOPER SOLUTION**

**RELATED APPLICATION**

This is a Divisional Application of application Ser. No. 08/703,593, filed Aug. 27, 1996 which a Continuation-in-part Application of application Ser. No. 08/590,241, filed Jan. 23, 1996, both were abandoned.

**FIELD OF THE INVENTION**

The present invention relates to the processing of silver bromoiodide color negative films. In particular, it relates to color development of such films at high temperatures using heat stabilized color developer solutions having a specific hydroxylamine antioxidant.

**BACKGROUND OF THE INVENTION**

Production of photographic color images from light sensitive materials basically consists of two processes. First, color negative images are generated by light exposure of camera speed light sensitive films, which are sometimes called "originating" elements because the images are originated therein by the film user (that is, "picture taker"). These negative images are then used to generate positive images in light sensitive materials having a reflective base using a "printer". These latter materials are sometimes known as "display" elements and the resulting images may be known as "prints" or motion picture projection films.

The light sensitive materials are processed in several steps and processing solutions to provide the necessary images in automatic processing machines. Traditionally, this service has required one or two days for providing the customer with the desired prints. In recent years, customers have wanted faster service, and in some locations known as "mini-labs", it is desired to provide the customer with the desired prints within an hour. This requires the photoprocessing methods to be even faster, and reducing the processing time to within a few minutes is the ultimate desire in the industry.

Reduction in processing time of the "display" elements or color photographic papers has been facilitated by a number of recent innovations, including the use of predominantly silver chloride emulsions in the display elements.

Color negative films generally comprise little or no silver chloride in their emulsions, and generally have silver bromide as the predominant silver halide. More typically, the emulsions are silver bromoiodide emulsions with silver iodide levels up to several mol percent. Such films require these types of emulsions because emulsions containing high silver chloride have not demonstrated sufficient light sensitivity to be used as camera speed materials although they have the advantage of being rapidly processed without major changes to the color developer solution.

However, to shorten the processing time, specifically the color development time, of films containing silver bromoiodide emulsions, more active color developer solutions are needed. Various attempts have been made to increase color developer activity by increasing the pH, color developing agent concentration or temperature. However, when these changes are made, the stability of the solution often diminishes. For example, when the development temperature is increased from the conventional 37.8° C., and the color developer solution is held (or used) in the processing tanks

for extended periods of times, silver bromoiodide elements processed with such solutions often exhibit unacceptably high density in the unexposed areas of the elements, that is unacceptably high Dmin.

Various methods have been proposed for stabilizing color developer solutions during use, but these methods are primarily used in processing high silver chloride emulsions. For example, color developers in U.S. Pat. No. 4,876,174 as being stabilized for processing high silver chloride by containing dialkylhydroxylamine antioxidants or preservatives. Other preservatives are also described in the art, such as hydrazines, hydroxamic acid and alpha-hydroxyketones, as described for example in U.S. Pat. No. 4,897,339 and U.S. Pat. No. 4,906,554. Another method for stabilization is to use an anionic surface active agent in combination with a substituted alkylhydroxylamine to process high silver chloride elements having a dry thickness of less than 15  $\mu\text{m}$ , as described in U.S. Pat. No. 5,091,292. Still another method involves using a processor having a small surface ratio of the color developer so it has less contact with air.

All of the foregoing methods have been designed for processing high silver chloride photographic papers, and have not been shown to be effective in processing color negative silver bromoiodide films.

Attempts have also been made to stabilize color developing solutions prior to their use, by storing them in sealed containers having low permeability to oxygen, as described in U.S. Pat. No. 4,814,260. Components that produce gases in the solutions are removed or replaced by non-gas producing components. Other storage containers have been designed from multilayers of various polymeric materials to reduce oxygen transmittance. However, these attempts fail to provide stability when the color developer solutions are being held for long periods of time at high temperature in the processing machine, especially when development is carried out at high temperature.

There remains a need for a process for rapid color development of silver bromoiodide films using color developer solutions stabilized for high temperature keeping.

**SUMMARY OF THE INVENTION**

The problems described above have been overcome with a method of photoprocessing comprising:

A) color developing an imagewise exposed color negative photographic film element containing at least one silver bromoiodide emulsion, with a color developer solution that comprises:

a color developing agent present at from about 0.01 to about 0.1 mol/l, and

an antioxidant present at from about 0.001 to about 0.5 mol/l, the antioxidant having the formula:



wherein L and L' are independently alkylene of 1 to 8 carbon atoms or alkylenephenylene of 1 to 3 carbon atoms in the alkylene portion, and R and R' are independently hydrogen, carboxy, sulfo or phosphono, provided that at least one of R and R' is not hydrogen,

the contacting being carried out at from about 45 to about 65° C. for from about 20 to about 150 seconds, provided that the photographic film element exhibits

a  $\Delta\text{Dmin}$  of less than 10% when processed with the color developer solution that has been held at 57.5° C. for up to 320 hours prior to processing.

This invention also provides a method for stabilizing a color developer solution comprising:

mixing a color developing agent present at from about 0.01 to about 0.1 mol/l, with an antioxidant present at from about 0.001 to about 0.5 mol/l, the antioxidant having the formula:



wherein L and L' are independently alkylene of 1 to 8 carbon atoms or alkylenephenylene of 1 to 3 carbon atoms in the alkylene portion, and R and R' are independently hydrogen, carboxy, sulfo or phosphono, provided that at least one of R and R' is not hydrogen,

provided that when the color developer solution is held at 57.5° C. for up to 320 hours, and is then used to process a color photographic film having at least one color record comprising a silver bromoiodide emulsion having associated therewith a color forming coupler, the  $\Delta D_{min}$  of the three color records will be less than 10% when the largest change in any color record is positive (that is, increasing  $D_{min}$ ) or less than 5% when the largest change in any color record is negative (that is, decreasing  $D_{min}$ ), wherein  $\Delta D_{min}$  is defined as:

$$\Delta D_{min} = \frac{(1\% Cr + 1\% Cg + 1\% Cb)}{3}$$

$$\% C_i = \left[ \frac{D_{min,i}(t) - D_{min,i}(0)}{D_{min,i}(0)} \right] \times 100$$

"i" is r (red), g (green), or b (blue) and "t" is time.

The method of this invention allows for rapid color development of camera ready film elements containing a silver bromoiodide emulsion. The color developer solutions are remarkably stable even when maintained and/or used at relatively high temperatures, that is, above 45° C. for lengthy periods of time. This stability is obtained by including in the color developer solutions a specific hydroxylamine derivative. While there are many hydroxylamines known as useful antioxidants in color developer solutions, it has been unexpectedly found that the combination of photographic elements having silver bromoiodide emulsions and color developer solutions containing the specific hydroxylamine derivatives described herein minimizes unacceptable increase in  $D_{min}$  when the color developer solutions are kept and used at high processing temperatures for extended periods of time.

The  $\Delta D_{min}$  increase in the color records of the elements is kept at 10% or less when such color developer solutions are maintained and/or used at elevated temperatures, such as 57.5° C. for up to 320 hours.

#### DETAILED DESCRIPTION OF THE INVENTION

The antioxidants useful in the practice are represented by the formula:



wherein L and L' are independently substituted or unsubstituted alkylene of 1 to 8 carbon atoms (such as methylene, ethylene, n-propylene, isopropylene, n-butylene, 1,1-dimethylethylene, n-hexylene, n-octylene and sec-butylene), or substituted or unsubstituted alkylenephenylene of 1 to 3 carbon atoms in the alkylene portion (such as benzylene, dimethylenephylene, and isopropylidenephylene).

The alkylene and alkylenephenylene groups can also be substituted with up to 4 substituents that do not interfere with the stabilizing effect of the molecule, or the solubility

of the compound in the color developer solution. Such substituents must be compatible with the color developer components and must not negatively impact the photographic processing system. Such substituents include but are not limited to, alkyl of 1 to 6 carbon atoms, fluoroalkyl groups of 1 to 6 carbon atoms, alkoxy of 1 to 6 carbon atoms, phenyl, hydroxy, halo, phenoxy, alkylthio of 1 to 6 carbon atoms, acyl groups, cyano, or amino.

In the noted formula, R and R' are independently hydrogen, carboxy, sulfo, phosphono, or other acid groups, provided that at least one of R and R' is not hydrogen. Salts of the acid groups are considered equivalents in this invention. Thus, the free acid forms of the hydroxylamines can be used, as well as the organic or inorganic salts of the acids, such as the alkali metal, pyridinium, tetraethylammonium, tetramethylammonium and ammonium salts. The sodium and potassium salts are the preferred salts. In addition, readily hydrolyzable ester equivalents can also be used, such as the methyl and ethyl esters of the acids. When L or L' is alkylenephenylene, the carboxy, sulfo or phosphono group is preferably at the para position of the phenylene, but can be at other positions if desired. More than one carboxy, sulfo or phosphono group can be attached to the phenylene radical.

Preferably, one or both of R and R' are hydrogen, carboxy or sulfo, with hydrogen and sulfo (or salts or readily hydrolyzable esters thereof) being more preferred. Most preferably, R is hydrogen and R' is sulfo (or a salt thereof).

Preferably, L and L' are independently substituted or unsubstituted alkylene of 3 to 6 carbon atoms (such as n-propyl, isopropyl, n-butyl, sec-butyl, t-butyl, n-pentyl, 1-methylpentyl and 2-ethylbutyl), or substituted or unsubstituted alkylenephenylene having 1 or 2 carbon atoms in the alkylene portion (such as benzyl, and dimethylenephene).

More preferably, at least one, and optionally both, of L and L' is a substituted or unsubstituted alkylene group of 3 to 6 carbon atoms that is branched at the carbon atom directly attached (that is, covalently bonded) to the nitrogen atom of the hydroxylamine molecule. Such branched divalent groups include, but are not limited to, isopropylene, sec-butylene, t-butylene, sec-pentylene, t-pentylene, sec-hexylene and t-hexylene. Isopropylene is most preferred.

In one embodiment, L and L' are the same. In other and preferred embodiments, they are different. In the latter embodiment, L is more preferably a branched alkylene as described above, and L' is a linear alkylene of 1 to 6 carbon atoms (such as methylene, ethylene, n-propylene, n-butylene, n-pentylene and n-hexylene).

Representative hydroxylamine derivatives useful in the practice of this invention include, but are not limited to, N-isopropyl-N-(2-ethanesulfonic acid)hydroxylamine, N,N-bis(propionic acid)hydroxylamine, N,N-bis(2-ethanesulfonic acid)hydroxylamine, N-isopropyl-N-(n-propylsulfonic acid)hydroxylamine, N-2-ethanephosphonic acid-N-(propionic acid)hydroxylamine, N,N-bis(2-ethanephosphonic acid)hydroxylamine, N-sec-butyl-N-(2-ethanesulfonic acid)hydroxylamine, N,N-bis(sec-butylcarboxylic acid)hydroxylamine, N-methyl-N-(p-carboxylbenzyl)hydroxylamine, N-isopropyl-N-(p-carboxylbenzyl)hydroxylamine, N,N-bis(p-carboxylbenzyl)hydroxylamine, N-methyl-N-(p-carboxyl-m-methylbenzyl)hydroxylamine, N-isopropyl-N-(p-sulfonylbenzyl)hydroxylamine, N-ethyl-N-(p-phosphonobenzyl)hydroxylamine, N-isopropyl-N-(2-carboxymethylene-3-propionic acid)hydroxylamine, and alkali metal salts thereof. The first compound and the sodium or potassium salts thereof are most preferred.

The hydroxylamine derivatives described herein as useful antioxidants can be readily prepared using published

procedures, such as those described in U.S. Pat. No. 3,287,125, U.S. Pat. No. 3,778,464, U.S. Pat. No. 5,110,985 and U.S. Pat. No. 5,262,563, all incorporated herein by reference for the synthetic methods. One general synthetic procedure for preparing sulfo-substituted hydroxylamines derivatives comprises reacting an N-alkylhydroxylamine with a vinylsulfonate in a suitable solvent (such as water, an alcohol, tetrahydrofuran or methyl ethyl ketone). For the alkali metal salts of vinylsulfonates, water is the best solvent. In cases where the hydroxylammonium salt is available, an equivalent of a base must be used to liberate the free N-alkylhydroxylamine. Commercial sources of free N-alkylhydroxylamines and N-alkylhydroxylammonium salts include Angus Chemicals and Aldrich Chemical Company. Further details of this procedure would be readily apparent to one skilled in the art.

To prepare the compounds having alkylenephenylene groups, a mono-substituted hydroxylamine can be reacted with  $\alpha$ -halo-toluic acids (or equivalent substituted  $\alpha$ -halotoluic acids), as further described in copending and commonly assigned U.S.S.N. 08/448,075 filed May 23, 1995, by Marrese et al as a Continuation of U.S.S.N. 08/257,601 on Jun. 9, 1994, now abandoned.

An alternative synthetic preparation method comprises reacting a vinylic compound having the structure



with a hydroxylamine having the structure HO—NHR<sub>5</sub>, wherein R<sub>1</sub> and R<sub>2</sub> are independently hydrogen or an alkyl group, R<sub>3</sub> is hydrogen, halo or an alkyl group, and R<sub>4</sub> is sulfo, —COOR<sub>7</sub> wherein R<sub>7</sub> is hydrogen or an alkyl group of 1 to 4 carbon atoms, or phosphono. R<sub>5</sub> is hydrogen, an



alkyl group of 1 to 12 carbon atoms or, the reacting step taking place in water or a water-miscible organic solvent, or mixture thereof, in the absence of a neutralizing base.

Useful solvents for this reaction include lower alcohols (such as methanol, ethanol or isopropanol) or other water-miscible solvents (such as N-methyl pyrrolidone, tetrahydrofuran, N, N-dimethylacetamide, N, N-dimethylformamide or dimethylsulfoxide), or mixtures of any of these solvents (with or without water). The reaction temperature can be from about 0 to about 100° C., and will take generally at least two hours. The reaction mixture can have any desirable pH less than about 10.

Specific preparations of preferred compounds are described below prior to the Examples for illustrative purposes. The compounds for which a synthesis is not described can be similarly prepared using routine modifications that would be readily apparent to one skilled in the art.

The antioxidant described herein is included in the color developer solution in an amount of at least about 0.001 mol/l, and in a preferred amount of from about 0.001 to about 0.5 mol/l. A most preferred amount is from about 0.005 to about 0.5 mol/l. More than one antioxidant can be used in the same color developer solution if desired, but preferably, only one is used.

The pH of the color developer solution is generally from about 9 to about 12 (preferably from about 10 to about 11), as provided by the addition of one or more weak or strong bases (such as a hydroxide) or buffers in amounts readily known in the art. Particularly useful buffers include, but are not limited to, carbonates, borates, tetraborates, phosphates, glycine salts, leucine salts, valine salts, proline salts, alanine salts, aminobutyric acid salts, lysine salts, guanine salts and hydroxybenzoates.

The color developer solutions include one or more color developing agents, of which there are hundreds of possibilities. Useful classes of such materials include, but are not limited to, aminophenols, p-phenylenediamines (especially N,N-dialkyl-p-phenylenediamines) and others that are well known in the art, such as EP 0 434 097A1 (published Jun. 26, 1991) and EP 0 530 921A1 (published Mar. 10, 1993). It may be useful for the color developing agents to have one or more water-solubilizing groups as are known in the art. Further details of such materials are provided in *Research Disclosure*, publication 36544, pages 501-541 (September 1994). *Research Disclosure* is a publication of Kenneth Mason Publications Ltd., Dudley House, 12 North Street, Emsworth, Hampshire PO10 7DQ England (also available from Emsworth Design Inc., 121 West 19th Street, New York, N.Y. 10011). This reference will be referred to hereinafter as "*Research Disclosure*". Generally, the amount of color developing agent is from about 0.01 to about 0.1 mol/l, with from about 0.02 to about 0.06 mol/l being preferred.

The color developer solution can be easily prepared by mixing a suitable color developing agent (in a suitable solution) with an antioxidant as described above (in a suitable aqueous solution). Water can be added to the resulting solution to provide the desired concentrations of an aqueous solution, and the pH can be adjusted as noted above.

The solution can also include one or more of a variety of other addenda which are commonly used in such compositions, such as alkali metal halides (such as potassium chloride, potassium bromide, sodium bromide and sodium iodide), metal sequestering agents (such as polycarboxylic or aminopolycarboxylic acids or polyphosphonates), buffers (as noted above), other preservatives (such as sulfites and alcoholamines), antifoggants, development accelerators, optical brighteners, wetting agents, stain reducing agents, surfactants, defoaming agents, and water-soluble or water-dispersible color couplers, as would be readily understood by one skilled in the art (see for example, *Research Disclosure*, noted above and U.S. Pat. No. 4,814,260 of Koboshi et al). The amounts of such additives are well known in the art also. For example, the amounts of halides can be varied widely, but are generally at least about  $5 \times 10^{-5}$  to about 0.4 mol/l for bromide ion and at least about  $5 \times 10^{-7}$  and up to about 0.01 mol/l for iodide ion. A preferred color developing composition is described below in Example 1. The color developing solution may or may not contain chloride ion because chloride ion essentially has no effect on the efficacy of the color developer composition. Thus, generally, chloride ion is not added or present, but if it is, it is not detrimental to the invention. It is more important that some bromide and iodide ions be present in the color developer solution.

While other known preservatives such as sulfites or alcohol amines (such as triethandiamine) can be present, the color developer solution contains no hydroxylamine or hydroxylamine derivatives besides those described above.

The color developing solution is preferably formulated and used as an aqueous solution, either as the working developer solution or as a replenishing solution. However, as is known in the art, they can also be formulated and used as

dry tablets. The technology for this is readily known in the art, such as U.S. Pat. No. 5,362,610 (Yoshimoto), U.S. Pat. No. 5,376,509 (Yoshimoto et al) and EP-A-0 611 986A1 (published Aug. 24, 1994).

The color developing solution has obvious utility to provide color development of an imagewise exposed color photographic negative image forming film element comprising a support and one or more silver halide emulsion layers (or color records) containing an imagewise distribution of developable silver halide emulsion grains, and having one or more color forming couplers associated therewith. A wide variety of types of photographic films containing various types of emulsions can be processed using the present invention, the types of elements being well known in the art (see *Research Disclosure*, noted above). The color developer solution can also be used in the processing of color reversal films having one or more color records.

The present invention is particularly useful for processing camera speed negative photographic films containing silver bromoiodide emulsions. Generally, the iodide content of such silver halide emulsions is less than about 40 mol % (based on total silver), preferably from about 0.05 to about 10 mol %, and more preferably, from about 0.5 to about 6 mol %. The emulsions can be of any crystal morphology (such as cubic, octahedral, cubooctahedral or tabular as are known in the art), or irregular morphology (such as multiple twinning or rounded). Preferably, the elements have at least two separate light sensitive emulsion layers, and each layer contains a silver bromoiodide emulsion as defined above.

Such elements generally have a camera speed defined as an ISO speed of at least 25, and preferably an ISO speed of at least 50.

The speed or sensitivity of color negative photographic materials is inversely related to the exposure required to enable the attainment of a specified density above fog after processing. Photographic speed for color negative films with a gamma of about 0.65 has been specifically defined by the American National Standards Institute (ANSI) as ANSI Standard Number PH 2.27-1979 (ASA speed) and relates to the exposure levels required to enable a density of 0.15 above fog in the green light sensitive and least sensitive recording unit of a multicolor negative film. This definition conforms to the International Standards Organization (ISO) film speed rating.

The layers of the photographic elements can have any useful binder material or vehicle known in the art, including various types of gelatins and other colloidal materials (or mixtures thereof). One useful binder material is acid processed gelatin that can be present in any layer in any suitable amount.

The elements are typically exposed to suitable radiation to form a latent image and then processed to form a visible dye image. Processing includes the step of color development in the presence of a color developing agent (typically in a color developer) to reduce developable silver halide and to oxidize the color developing agent. Oxidized color developing agent in turn reacts with a color-forming coupler to yield a dye. Silver in the element can then be removed using conventional bleaching and fixing solutions.

Development is carried out by contacting the element under suitable time and temperature conditions, in suitable processing equipment, to produce the desired developed image. Additional processing steps can then be carried out using conventional procedures, including but not limited to, one or more development stop, bleaching, fixing, washing (or rinsing), stabilizing and drying steps, in any particular desired order as would be known in the art for either color

negative or color reversal processing methods. Useful processing steps, conditions and materials useful therefor are well known (see for example, *Research Disclosure*).

The photographic elements processed in the practice of this invention can be single or multilayer color elements. Multilayer color elements typically contain dye image-forming units (or color records) sensitive to each of the three primary regions of the visible spectrum. Each unit can be comprised of a single emulsion layer or multiple emulsion layers sensitive to a given region of the spectrum. The layers of the element can be arranged in any of the various orders known in the art. In an alternative format, the emulsions sensitive to each of the three primary regions of the spectrum can be disposed as a single segmented layer. The elements can also contain other conventional layers such as filter layers, interlayers, subbing layers, overcoats and other layers readily apparent to one skilled in the art. A magnetic backing can be used as well as conventional supports.

Considerable details of the element structure and components, and suitable methods of processing various types of elements are described in *Research Disclosure*, noted above. Included within such teachings in the art is the use of various classes of cyan, yellow and magenta color couplers which can be used with the present invention. In particular, the present invention can be used to process photographic elements containing pyrazolotriazole magenta dye forming couplers.

Representative color negative films that can be processed using the present invention include, but are not limited to, KODAK ROYAL GOLD® films, KODAK GOLD® PLUS 100 film, KODAK GOLD® SUPER 200 film, KODAK GOLD ULTRA 400 film, FUJI SUPER G Plus films, FUJI SMARTFILM™ products, KONICA VX films, KONICA SRG3200 film, 3M SCOTCH® ATG films, and AGFA HDC and XRS films.

Processing according to the present invention can be carried out using conventional deep tanks holding processing solutions or automatic processing machines. Alternatively, it can be carried out using what is known in the art as "low volume thin tank" processing systems, or LVT, which have either a rack and tank or automatic tray design. Such processing methods and equipment are described, for example, in U.S. Pat. No. 5,436,118 (Carli et al) and publications noted therein.

The length of time and temperatures used for each processing step of the present invention, other than color development, can be any desired condition, whether conventional or not.

The color developer solutions described herein are stable when stored and/or used at the elevated temperatures described herein for extended periods of time, for example up to 300 hours. Typically, such temperatures are encountered during rapid photoprocessing methods where the silver bromoiodide films described above are color developed after imagewise exposure.

For color development, the processing temperature is generally from about 45° to about 65° C., preferably from about 50° to about 65° C., and more preferably from about 50° to about 60° C. Most preferably, the development temperature is from about 55 to about 60° C.

The time for color development is from about 20 to about 150 seconds, with a time of from about 30 to about 120 seconds being preferred, and a time of from about 30 to about 90 seconds being more preferred. The overall processing time (from development to final rinse or wash) can be from about 50 seconds to about 40 minutes. Shorter overall processing times, that is, less than about 3 minutes,

are desired for processing photographic color negative films according to this invention.

A preferred embodiment of this invention is a method of photoprocessing comprising:

A) color developing an imagewise exposed color negative photographic film element containing a red-sensitive emulsion layer, a green-sensitive emulsion layer and a blue-sensitive emulsion layer, each emulsion layer comprising a silver bromoiodide emulsion comprising from about 0.5 to about 10 mol % iodide based on total silver,

with a color developer solution that comprises:

a color developing agent present at from about 0.01 to about 0.1 mol/l, and

an antioxidant present at from about 0.001 to about 0.5 mol/l, the antioxidant having the formula:



wherein L and L' are independently alkylene of 3 to 5 carbon atoms, at least one of L and L' being an alkylene that is branched at the carbon atom attached to the nitrogen atom, and R and R' are independently hydrogen, carboxy or sulfo, provided that at least one of R and R' is not hydrogen,

the color developing being carried out at from about 50 to about 60° C. for from about 30 to about 90 seconds, provided that the photographic film element exhibits a  $\Delta D_{min}$  of less than 10% when processed with the color developer solution that has been held at 57.5° C. for up to 320 hours prior to processing,

B) bleaching the color developed element,

C) fixing the bleached element, and

D) washing or rinsing the fixed element.

The following synthetic preparations and examples are provided to illustrate preparation of several preferred hydroxylamines, as well as the practice of this invention and not to limit it in any way. Unless otherwise indicated, percentages are by weight.

#### Preparation of N-isopropyl-N-(2-ethanesulfonic acid) hydroxylamine

Isopropyl hydroxylamine (330 g of 15% in water, 0.665 mol) was combined with sodium vinylsulfonate (350 g of 25% in water, 0.665 mol) and sodium hydroxide (0.4 g, 0.01 mol). The resulting solution was refluxed for four hours, after which no starting materials were detected by thin layer chromatography. The reaction mixture was cooled to room temperature and precipitated into eight liters of stirred isopropanol. The resulting white solid was dried in a vacuum oven prior to use.  $^1H$ NMR ( $\delta$ , ppm) 2.9–3.1 (br,  $CH_2CH_2$ , 4H), 2.85 (septet, i-Pr, 1H), 0.95(d, i-Pr, 6H) confirmed the structure, and ion chromatography revealed no chloride ion and 1.2% sulfate.

#### Preparation of N-isopropyl-N-(2-ethanesulfonic acid)hydroxylamine, Sodium Salt

An aqueous solution (420 ml) of vinylsulfonic acid, sodium salt (25%) was heated to reflux. While at reflux, an aqueous solution (480 g) of isopropyl hydroxylamine was linearly added over a period of two hours. During the next five hours, water (600 g) was removed linearly by distillation. After cooling the reaction solution to 20° C., isopropanol (500 ml) was added with good mechanical stirring to keep the resulting white solid suspended. This solid was collected on a sintered glass funnel, rinsed with additional fresh isopropanol (100 ml), and dried overnight at 50° C. under vacuum for analysis. N-isopropyl-N-(2-

ethanesulfonic acid)-hydroxylamine, sodium salt was isolated as a white powder. However, the product could have been left in the reaction solution for later use if desired.

All analyses were consistent with the structure of the desired compound. The  $^1H$  NMR in  $D_2O$  had peaks at 4.8(NOH), 3.2–2.9(isopropyl methine and two methylenes of the ethylsulfonato sodium salt moiety), and 1.1 ppm (two methyls of the isopropyl group). The  $^{13}C$  NMR had peaks at 59.4, 52.4, 49.9 and 19.2 ppm. The sodium analysis was 11.5%.

#### Preparation of Bis(2-ethanesulfonic acid) hydroxylamine, Disodium Salt

An aqueous solution (150 ml) of vinylsulfonic acid, sodium salt (25%) was heated to 70° C. over a period of 30 minutes. While the solution was stirred, an aqueous solution (10.3 g) of hydroxylamine (50%) was linearly added over a period of 5 minutes. The reaction solution was held at 70° C. for eight hours, then cooled to 20° C. over a period of 30 minutes. To the reaction solution was then added methanol (800 ml) over a period of 5 minutes. After an additional 30 minutes, the resulting solid product was collected on a filter funnel, rinsed with fresh methanol (100 ml), and dried overnight at 50° C. under vacuum to give 49 g of white solid for analysis.

The analyses were consistent with the structure of the desired product. The  $^1H$  NMR in  $D_2O$  had peaks at 4.8 (NOH), and 4.7 and 3.2 ppm for the two different methylene protons in the molecule. The  $^{13}C$  NMR had peaks at 56.4 and 49.8 ppm for the methylene carbons in the molecule. The sodium analysis was 15.1% (consistent for the monohydrate).

#### Preparation of N-isopropyl-N-(3-propionic Acid) hydroxylamine

Acrylic acid (120 g) was added to an aqueous solution (825 g) of isopropylhydroxylamine (15%) and methanol (1250 ml) at room temperature with vigorous mechanical stirring. Upon completion of the addition, the reaction solution was heated to 60° C. and maintained at that temperature overnight. Upon cooling to room temperature and concentration of the reaction solution by evaporation, a yellow oil crystallized upon standing. Isopropanol and ether were added to facilitate collection of the resulting product by suction filtration for analysis. The resulting white granular solid was dried overnight under vacuum to give 155 g.

The analyses were consistent with the desired structure. The  $^1H$  NMR in dimethylsulfoxide-d6 had peaks at 7.0 (NOH), 2.7(isopropyl methine plus methylene group of-the propionic acid moiety), 2.35(methylene of propionic acid moiety), and 0.9 ppm(two methyls of the isopropyl group). The mass spectrum was consistent with the desired compound.

#### Preparation of Bis-N-(2-carboxyethyl) hydroxylamine, Dimethylester

Methanol (200 ml) was added to a mechanically stirred aqueous solution of hydroxylamine (13.24 g of 50% solution, 0.2 moles). Methyl acrylate (34.44 ml, 0.4 moles) was added dropwise to the solution at 25° C. over thirty minutes as the solution became warm during the resulting

reaction. After completion of the addition, the reaction mixture was heated to 60° C. in an oil bath and stirred overnight. The pH of the resulting mixture was 6.15. The solution was then cooled to room temperature, and concentrated at 40° C. under reduced pressure to yield a pale yellow, cloudy oil (41.6 g, 99%).

All analyses of the oil were consistent with the desired structure. The <sup>1</sup>H NMR spectrum in dimethylsulfoxide-d6 had peaks at 7.9 (NOH), 3.54 (s,6H), 2.75 (t,4H), and 2.45 (t,4H).

#### Preparation of Bis-N-(2-Carboxyethyl) hydroxylamine, Diethylester

Methanol (200 ml) was added to a mechanically stirred aqueous solution of hydroxylamine (13.24 g of 50% solution, 0.2 moles). Ethyl acrylate (43.34 ml, 0.4 moles) was added dropwise to the solution at 25° C. over thirty minutes as the solution became warm during the resulting reaction. After completion of the addition, the reaction mixture was heated to 60° C. in an oilbath and stirred overnight. The pH of the resulting mixture was 6.5. The solution was then cooled to room temperature, and concentrated at 40° C. under reduced pressure to yield a pale yellow, cloudy oil (46.3 g, 99%).

All analyses of the oil were consistent with the desired structure. The <sup>1</sup>H NMR spectrum in dimethylsulfoxide-d6 had peaks at 7.9 (NOH), 4.0 (q,4H), 2.75 (t,4H), 2.40 (t,4H), and 1.1 (t,6H).

#### Preparation of N-(2-carboxyethyl)-N-hydroxy-β-Alanine

Methanol (200 ml) was added to a mechanically stirred aqueous solution of hydroxylamine (13.24 g of 50% solution, 0.2 moles). Acrylic acid (27.4 ml, 0.4 moles) was added dropwise to the solution at 25° C. over thirty minutes. After a few hours of reaction, a white precipitate began to form. The reaction mixture was stirred overnight at room temperature, and the resulting white solid was filtered out, washed with cold water, and dried in vacuum overnight to give 30.4 g (85%) of the desired compound.

All analyses of the solid were consistent with the desired structure. The <sup>1</sup>H NMR spectrum in dimethylsulfoxide-d6 had peaks at 5.0 (br.s), 2.7 (t,4H) and 2.35 (t,4H), and a melting point of 148°–149° C.

#### Preparation of N-isopropyl-N-(2-carboxymethylene-3-propionic acid)-hydroxylamine

Methanol (300 ml) was added to an aqueous 15% solution (400 ml) of N-isopropylhydroxylamine (0.8 moles), followed by addition of itaconic acid (104 g, 0.8 moles) in portions as a solid. Additional methanol (100 ml) was used to rinse the itaconic acid into the flask. After all of the solid acid had dissolved, the mixture was stirred at room temperature for 6 days, and filtered to collect the resulting white solid product. This material was dried under mild vacuum to a weight of 142 g (m.p. 136°–8° C.). NMR analysis was consistent with the structure of the desired compound.

Similarly, bis(2-carboxymethylene-3-propionic acid) hydroxylamine was prepared using similar conditions and slightly varying solvent mixtures of water and methanol, water and tetrahydrofuran or tetrahydrofuran and N,N-dimethylformamide. This compound was prepared by reacting itaconic acid with hydroxylamine.

#### Materials and Methods for the Examples

The following stock color developer solution was used in the following Comparative and Invention Examples:

|                                                                    |        |
|--------------------------------------------------------------------|--------|
| Potassium carbonate, anhydrous                                     | 34.3 g |
| Potassium bicarbonate                                              | 2.32 g |
| Sodium sulfite, anhydrous                                          | 0.38 g |
| Sodium metabisulfite                                               | 2.78 g |
| Potassium iodide                                                   | 1.2 mg |
| Sodium bromide                                                     | 1.3 g  |
| Diethylenetriaminepentaacetic acid, pentasodium salt               | 3.37 g |
| Hydroxylamine antioxidant                                          | 2.41 g |
| Ethanol,2-[[(4-amino-3-methyl-phenyl)ethylamino]sulfate (1:1) salt | 4.52 g |
| Water to make 1 liter (pH adjusted to 10.0)                        |        |

The following examples show the magnitude of changes in the minimum (Dmin) and maximum (Dmax) density regions in each color record of imagewise exposed, processed commercially available KODAK GOLD ULTRA™ 400 speed color negative film as a function of the color developer age, temperature and antioxidant. The film samples used in Comparative Example 1 were developed at the standard temperature of 37.8° C. for 3 minutes and 15 seconds using the commercially known KODAK C-41 RA processing method (including development, bleaching, fixing and rinsing). All other examples were developed for 45 seconds at 57.5° C. (unless otherwise noted).

The percent density changes for each color record (identified as "%Cr" for red record, "%Cg" for green record, and "%Cb" for blue record) were calculated as:

$$\% C_{Dmin} = \{[Dmin(t) - Dmin(0)]/Dmin(0)\} \times 100, \text{ or}$$

$$\% C_{Dmax} = \{[Dmax(t) - Dmax(0)]/Dmax(0)\} \times 100.$$

wherein Dmin(t) and Dmax(t) are the densities at time "t" after the experiments have begun, and Dmin(0) and Dmax(0) are the densities at the start of the experiments. By color records is meant the red-, green- and blue-sensitive units in the film samples, each unit having one or more emulsion layers having the desired light sensitivity.

#### COMPARATIVE EXAMPLE 1

In this experiment, which is representative of the commercial C-41 Process, the color developer solution contained hydroxylamine sulfate as the antioxidant. Tables I and II show the results of density changes in each color record of the processed film samples for given "aging" times (time at 37.8° C.) of color developer solution.

TABLE I

| Time (Hours) | Dmin Red Record | Dmin Green Record | Dmin Blue Record | % Cr  | % Cg | % Cb |
|--------------|-----------------|-------------------|------------------|-------|------|------|
| 0            | 0.257           | 0.695             | 0.951            | 0.00  | 0.00 | 0.00 |
| 48           | 0.260           | 0.669             | 0.955            | 1.17  | 0.58 | 0.42 |
| 120          | 0.261           | 0.701             | 0.957            | 1.56  | 0.86 | 0.63 |
| 168          | 0.260           | 0.701             | 0.954            | 1.17  | 0.86 | 0.32 |
| 196          | 0.252           | 0.697             | 0.952            | -1.29 | 0.29 | 0.11 |
| 223          | 0.256           | 0.699             | 0.955            | -0.39 | 0.58 | 0.42 |
| 288          | 0.258           | 0.702             | 0.952            | 0.39  | 1.01 | 0.11 |

TABLE II

| Time<br>(Hours) | Dmax Red<br>Record | Dmax<br>Green<br>Record | Dmax<br>Blue<br>Record | % Cr  | % Cg  | % Cb  |
|-----------------|--------------------|-------------------------|------------------------|-------|-------|-------|
| 0               | 1.18               | 1.71                    | 1.97                   | 0.00  | 0.00  | 0.00  |
| 48              | 1.18               | 1.69                    | 1.94                   | 0.00  | -1.17 | -1.52 |
| 120             | 1.19               | 1.70                    | 1.95                   | 0.85  | -0.58 | -1.02 |
| 168             | 1.18               | 1.69                    | 1.91                   | 0.00  | -1.17 | -3.05 |
| 196             | 1.15               | 1.67                    | 1.88                   | -2.54 | -2.34 | -4.57 |
| 223             | 1.17               | 1.68                    | 1.89                   | -0.85 | -1.75 | -4.06 |
| 288             | 1.15               | 1.65                    | 1.86                   | -2.54 | -3.51 | -5.58 |

The data in Tables I and II show that the standard C-41 Process conditions do not produce large changes in any of the color record densities. The largest positive change in Dmin is about 1% as represented by the change in the green record after aging the color developer for 288 hours. The Dmax in all three color records decreased as the color developer was aged, with the largest change being seen in the blue record at 288 hours. The loss of Dmax reflects a loss in color developer activity as a function of color developer solution hold time and is most probably due to the oxidation of the color developing agent by oxygen as the sulfite and hydroxylamine sulfate stabilizing agents are lost to oxidation.

## COMPARATIVE EXAMPLE 2

This experiment used the same processing solution compositions as in Comparative Example 1 except that the processing solutions were aged at 57.5° C. for extended periods of time. The changes in densities in the color records are shown in Tables III and IV below.

TABLE III

| Time<br>(Hours) | Dmin Red<br>Record | Dmin<br>Green<br>Record | Dmin Blue<br>Record | % Cr  | % Cg  | % Cb  |
|-----------------|--------------------|-------------------------|---------------------|-------|-------|-------|
| 0               | 0.304              | 0.735                   | 1.042               | 0.00  | 0.00  | 0.00  |
| 24              | 0.294              | 0.751                   | 1.044               | -3.29 | -1.90 | 0.19  |
| 96              | 0.321              | 0.760                   | 1.107               | 5.59  | 3.40  | 6.24  |
| 120             | 0.318              | 0.758                   | 1.110               | 4.61  | 3.13  | 6.53  |
| 144             | 0.332              | 0.768                   | 1.133               | 9.21  | 4.49  | 8.73  |
| 168             | 0.338              | 0.766                   | 1.141               | 11.18 | 4.22  | 9.50  |
| 264             | 0.393              | 0.816                   | 1.226               | 29.28 | 11.02 | 17.66 |
| 312             | 0.389              | 0.808                   | 1.227               | 27.96 | 9.93  | 17.75 |

TABLE IV

| Time<br>(Hours) | Dmax Red<br>Record | Dmax<br>Green<br>Record | Dmax<br>Blue<br>Record | % Cr  | % Cg | % Cb |
|-----------------|--------------------|-------------------------|------------------------|-------|------|------|
| 0               | 1.36               | 2.52                    | 3.37                   | 0.00  | 0.00 | 0.00 |
| 24              | 1.37               | 2.52                    | 3.38                   | 0.74  | 0.00 | 0.30 |
| 96              | 1.40               | 2.59                    | 3.46                   | 2.94  | 2.78 | 2.67 |
| 120             | 1.39               | 2.59                    | 3.47                   | 2.21  | 2.78 | 2.97 |
| 144             | 1.42               | 2.63                    | 3.54                   | 4.41  | 4.37 | 5.04 |
| 168             | 1.36               | 2.58                    | 3.48                   | 0.00  | 2.38 | 3.26 |
| 264             | 1.28               | 2.62                    | 3.54                   | -5.88 | 3.97 | 5.04 |
| 312             | 1.26               | 2.61                    | 3.53                   | -7.35 | 3.57 | 4.75 |

It is apparent that after being aged at the higher temperature, the color developer solution loses stability and produces undesirable density increases in Dmin all color records. These changes are as high as 29% in the red record after the color developer solution had been used at the high temperature for 264 hours. The changes in Dmax of the three

color records were about the same as those observed in Comparative Example 1.

## COMPARATIVE EXAMPLE 3

In this experiment, no hydroxylamine was included in the color developer. Thus, the color developer was the same as in Comparative Example 1 with the omission of a hydroxylamine derivative antioxidant. Aging of the solution and color development were carried out as in Comparative Example 2, that is, at 57.5° C. The changes in densities in the color records are shown in Tables V and VI below.

TABLE V

| Time<br>(Hours) | Dmin Red<br>Record | Dmin<br>Green<br>Record | Dmin Blue<br>Record | % Cr   | % Cg  | % Cb  |
|-----------------|--------------------|-------------------------|---------------------|--------|-------|-------|
| 0               | 0.283              | 0.724                   | 0.988               | 0.00   | 0.00  | 0.00  |
| 24              | 0.282              | 0.716                   | 0.996               | -0.35  | -1.10 | -0.81 |
| 96              | 0.275              | 0.716                   | 0.985               | -2.83  | -1.10 | -0.30 |
| 120             | 0.265              | 0.703                   | 0.979               | -6.36  | -2.90 | -0.91 |
| 144             | 0.269              | 0.695                   | 0.984               | -4.95  | -4.01 | -0.40 |
| 168             | 0.265              | 0.701                   | 0.983               | -6.36  | -3.18 | -0.51 |
| 264             | 0.253              | 0.686                   | 0.977               | -10.60 | -5.25 | -1.11 |
| 312             | 0.251              | 0.684                   | 0.970               | -11.31 | -5.25 | -1.82 |

TABLE VI

| Time<br>(Hours) | Dmax Red<br>Record | Dmax<br>Green<br>Record | Dmax Blue<br>Record | % Cr   | % Cg   | % Cb   |
|-----------------|--------------------|-------------------------|---------------------|--------|--------|--------|
| 0               | 1.34               | 2.49                    | 3.24                | 0.00   | 0.00   | 0.00   |
| 24              | 1.31               | 2.46                    | 3.16                | -2.24  | -1.20  | -2.47  |
| 96              | 1.18               | 2.31                    | 2.89                | -11.94 | -7.23  | -10.80 |
| 120             | 1.17               | 2.29                    | 2.86                | -12.69 | -8.03  | -11.73 |
| 144             | 1.17               | 2.29                    | 2.88                | -12.69 | -8.03  | -11.73 |
| 168             | 1.12               | 2.25                    | 2.83                | -16.42 | -9.64  | -12.96 |
| 264             | 0.99               | 2.13                    | 2.68                | -26.12 | -14.46 | -17.28 |
| 312             | 0.88               | 1.93                    | 2.45                | -34.33 | -22.49 | -24.38 |

The data show that when the hydroxylamine antioxidant is omitted, no increase in Dmin is seen as a function of time. In fact, the Dmin and Dmax of all three records decreased, consistent with the oxidative loss of the color developing agent. This Comparative Example illustrates the need to stabilize the color developing agent.

## INVENTION EXAMPLE 1

In this example of the invention, N-isopropyl-N-(2-ethanesulfonic acid)hydroxylamine (0.026 mol/l was used as the antioxidant in the color developer instead of hydroxylamine sulfate. Aging and processing were carried out as described for Comparative Example 2. The results are shown in Tables VII and VIII below.

TABLE VII

| Time<br>(Hours) | Dmin Red<br>Record | Dmin<br>Green<br>Record | Dmin Blue<br>Record | % Cr  | % Cg | % Cb  |
|-----------------|--------------------|-------------------------|---------------------|-------|------|-------|
| 0               | 0.259              | 0.664                   | 0.979               | 0.00  | 0.00 | 0.00  |
| 24              | 0.252              | 0.668                   | 0.971               | -2.70 | 0.60 | -0.82 |
| 48              | 0.254              | 0.676                   | 0.968               | -1.93 | 1.81 | -1.12 |
| 120             | 0.262              | 0.686                   | 0.983               | 1.16  | 3.31 | 0.41  |
| 144             | 0.262              | 0.696                   | 0.981               | 1.16  | 4.82 | 0.20  |
| 192             | 0.266              | 0.704                   | 0.989               | 2.70  | 6.02 | 1.02  |
| 216             | 0.260              | 0.695                   | 0.987               | 0.39  | 4.67 | 0.82  |

TABLE VII-continued

| Time<br>(Hours) | Dmin Red<br>Record | Dmin<br>Green<br>Record | Dmin Blue<br>Record | % Cr | % Cg | % Cb |
|-----------------|--------------------|-------------------------|---------------------|------|------|------|
| 312             | 0.273              | 0.700                   | 0.994               | 5.41 | 5.42 | 1.53 |
| 360             | 0.265              | 0.700                   | 0.990               | 2.32 | 5.42 | 1.12 |
| 456             | 0.262              | 0.697                   | 0.986               | 1.16 | 4.97 | 0.72 |

TABLE X-continued

| Time<br>(Hours) | Dmax Red<br>Record | Dmax<br>Green<br>Record | Dmax<br>Blue<br>Record | % Cr  | % Cg | % Cb |
|-----------------|--------------------|-------------------------|------------------------|-------|------|------|
| 168             | 1.19               | 2.44                    | 3.08                   | -4.80 | 2.95 | 1.99 |
| 192             | 1.17               | 2.45                    | 3.12                   | -6.40 | 3.38 | 3.31 |
| 240             | 1.14               | 2.46                    | 3.12                   | -8.80 | 3.80 | 3.31 |
| 312             | 1.14               | 2.57                    | 3.19                   | -8.80 | 8.44 | 5.63 |

TABLE VIII

| Time<br>(Hours) | Dmax Red<br>Record | Dmax<br>Green<br>Record | Dmax<br>Blue<br>Record | % Cr  | % Cg  | % Cb  |
|-----------------|--------------------|-------------------------|------------------------|-------|-------|-------|
| 0               | 1.05               | 2.04                    | 2.62                   | 0.00  | 0.00  | 0.00  |
| 24              | 1.03               | 2.02                    | 2.59                   | -1.90 | -0.98 | -1.15 |
| 48              | 1.04               | 2.03                    | 2.58                   | -0.95 | -0.49 | -1.53 |
| 120             | 1.04               | 2.02                    | 2.54                   | -0.95 | -0.98 | -3.05 |
| 144             | 1.08               | 2.07                    | 2.61                   | 2.86  | 1.47  | -0.38 |
| 192             | 1.08               | 2.07                    | 2.58                   | 2.86  | 1.47  | -1.53 |
| 216             | 1.06               | 2.04                    | 2.55                   | 0.95  | 0.00  | -2.67 |
| 312             | 1.11               | 2.11                    | 2.66                   | 5.71  | 3.43  | 1.53  |
| 360             | 1.12               | 2.14                    | 2.69                   | 6.67  | 4.90  | 2.67  |
| 456             | 1.09               | 2.14                    | 2.68                   | 3.81  | 4.90  | 2.29  |

The results in Table VII show that the change in Dmin as a function of time is much improved relative to Comparative Example 2, in all color records. The small changes in Dmax as a function of time, as shown in Table VIII, demonstrate the stability of the color developer solution used in this invention.

#### INVENTION EXAMPLE 2

This example is like Invention Example 1 except that N,N-bis(propionic acid)hydroxylamine (0.029 mol/l) was used as the color developer antioxidant, and the concentration of sodium bromide was increased to 0.051 mol/l. Aging and processing were carried out like Comparative Example 2. The results of the changes in color record densities are shown in Tables IX and X below.

TABLE IX

| Time<br>(Hours) | Dmin Red<br>Record | Dmin<br>Green<br>Record | Dmin Blue<br>Record | % Cr  | % Cg  | % Cb  |
|-----------------|--------------------|-------------------------|---------------------|-------|-------|-------|
| 0               | 0.247              | 0.682                   | 0.953               | 0.00  | 0.00  | 0.00  |
| 24              | 0.257              | 0.692                   | 0.958               | 4.05  | 1.47  | 0.52  |
| 48              | 0.247              | 0.681                   | 0.954               | 0.00  | -0.15 | 0.10  |
| 72              | 0.247              | 0.690                   | 0.958               | 0.00  | 1.17  | 0.52  |
| 144             | 0.240              | 0.676                   | 0.949               | -2.83 | -0.88 | -0.42 |
| 168             | 0.237              | 0.695                   | 0.962               | -4.05 | 1.91  | 0.94  |
| 192             | 0.233              | 0.682                   | 0.957               | -5.67 | 0.00  | 0.42  |
| 240             | 0.235              | 0.706                   | 0.972               | -4.86 | 3.52  | 1.99  |
| 312             | 0.243              | 0.727                   | 0.989               | -1.62 | 6.60  | 3.78  |

TABLE X

| Time<br>(Hours) | Dmax Red<br>Record | Dmax<br>Green<br>Record | Dmax<br>Blue<br>Record | % Cr | % Cg | % Cb  |
|-----------------|--------------------|-------------------------|------------------------|------|------|-------|
| 0               | 1.25               | 2.37                    | 3.02                   | 0.00 | 0.00 | 0.00  |
| 24              | 1.26               | 2.41                    | 3.11                   | 0.80 | 1.69 | 2.98  |
| 48              | 1.28               | 2.40                    | 3.01                   | 2.40 | 1.27 | -0.33 |
| 72              | 1.28               | 2.41                    | 3.04                   | 2.40 | 1.69 | 0.66  |
| 144             | 1.25               | 2.39                    | 3.06                   | 0.00 | 0.84 | 1.32  |

The results in Table IX are much improved relative to Comparative Example 2 in all color records. There was no increase in Dmin as the color developer solution was aged and only a small loss of Dmax was observed over time.

#### COMPARATIVE EXAMPLE 4

In this example, which is outside the scope of this invention, N-isopropyl-N-propionamide hydroxylamine (0.029 mol/l) was used in place of hydroxylamine sulfate in the color developer solution, and sodium bromide was increased to 0.051 mol/l. Aging and processing were carried out in the same manner as Comparative Example 2. The results are shown in Tables XI and XII below.

TABLE XI

| Time<br>(Hours) | Dmin Red<br>Record | Dmin<br>Green<br>Record | Dmin Blue<br>Record | % Cr   | % Cg  | % Cb  |
|-----------------|--------------------|-------------------------|---------------------|--------|-------|-------|
| 0               | 0.298              | 0.688                   | 0.944               | 0.00   | 0.00  | 0.00  |
| 48              | 0.268              | 0.669                   | 0.949               | -10.07 | -2.76 | 0.53  |
| 72              | 0.257              | 0.659                   | 0.942               | -13.76 | -4.22 | -0.21 |
| 144             | 0.246              | 0.668                   | 0.946               | -17.45 | -2.91 | 0.21  |
| 168             | 0.243              | 0.684                   | 0.954               | -18.46 | -0.58 | 1.06  |
| 192             | 0.234              | 0.684                   | 0.955               | -21.48 | -0.58 | 1.17  |
| 216             | 0.231              | 0.687                   | 0.955               | -22.48 | -0.15 | 1.17  |
| 240             | 0.235              | 0.691                   | 0.965               | -21.14 | 0.44  | 2.22  |
| 312             | 0.228              | 0.707                   | 0.983               | -23.49 | 2.76  | 4.13  |

TABLE XII

| Time<br>(Hours) | Dmax Red<br>Record | Dmax<br>Green<br>Record | Dmax<br>Blue<br>Record | % Cr   | % Cg  | % Cb  |
|-----------------|--------------------|-------------------------|------------------------|--------|-------|-------|
| 0               | 1.31               | 2.48                    | 3.10                   | 0.00   | 0.00  | 0.00  |
| 48              | 1.31               | 2.43                    | 3.04                   | 0.00   | -2.02 | -1.94 |
| 72              | 1.28               | 2.40                    | 3.03                   | -2.29  | -3.23 | -2.26 |
| 144             | 1.24               | 2.37                    | 2.99                   | -5.34  | -4.44 | -3.55 |
| 168             | 1.20               | 2.46                    | 3.12                   | -8.40  | -0.81 | 0.65  |
| 192             | 1.15               | 2.43                    | 3.06                   | -12.21 | -2.02 | -1.29 |
| 216             | 1.11               | 2.45                    | 3.04                   | -15.27 | -1.21 | -1.94 |
| 240             | 1.15               | 2.45                    | 3.07                   | -12.21 | -1.21 | -0.97 |
| 312             | 1.05               | 2.43                    | 2.99                   | -19.85 | -2.02 | -3.55 |

It is apparent from these results that the hydroxylamine derivative failed to prevent large changes in both Dmin and Dmax, especially in the red color record, as the color developer solution was aged. The direction and magnitude of the changes would suggest that the hydroxylamine derivative was not functioning as an effective antioxidant in this instance.

#### COMPARATIVE EXAMPLE 5

In this experiment, N,N-bis(propionamide) hydroxylamine (0.029 mol/l) was used as the antioxidant in the color developer solution, and the sodium bromide concentration was increased to 0.051 mol/l. Processing was

conducted as described in Comparative Example 2. The resulting density changes are shown in Tables XIII and XIV below.

TABLE XIII

| Time<br>(Hours) | Dmin<br>Red<br>Record | Dmin<br>Green<br>Record | Dmin Blue<br>Record | % Cr   | % Cg  | % Cb  |
|-----------------|-----------------------|-------------------------|---------------------|--------|-------|-------|
| 0               | 0.354                 | 0.705                   | 0.978               | 0.00   | 0.00  | 0.00  |
| 24              | 0.360                 | 0.731                   | 0.992               | 1.69   | 3.69  | 1.43  |
| 48              | 0.351                 | 0.716                   | 0.984               | -0.85  | 1.56  | 0.61  |
| 72              | 0.335                 | 0.728                   | 0.985               | -5.37  | 3.26  | 0.72  |
| 144             | 0.263                 | 0.690                   | 0.959               | -25.71 | -2.13 | -1.94 |
| 168             | 0.244                 | 0.698                   | 0.962               | -31.07 | -0.99 | -1.64 |
| 192             | 0.238                 | 0.688                   | 0.962               | -32.77 | -2.41 | -1.64 |
| 216             | 0.255                 | 0.698                   | 0.976               | -27.97 | -0.99 | -0.20 |
| 240             | 0.233                 | 0.705                   | 0.969               | -34.18 | 0.00  | -0.92 |
| 312             | 0.241                 | 0.726                   | 0.989               | -31.92 | 2.98  | 1.12  |

TABLE XIV

| Time<br>(Hours) | Dmax<br>Red<br>Record | Dmax<br>Green<br>Record | Dmax Blue<br>Record | % Cr   | % Cg  | % Cb  |
|-----------------|-----------------------|-------------------------|---------------------|--------|-------|-------|
| 0               | 1.31                  | 2.46                    | 3.05                | 0.00   | 0.00  | 0.00  |
| 24              | 1.31                  | 2.49                    | 3.05                | 0.00   | 1.22  | 0.00  |
| 48              | 1.41                  | 2.58                    | 3.28                | 7.63   | 4.88  | 7.54  |
| 72              | 1.35                  | 2.54                    | 3.19                | 3.05   | 3.25  | 4.59  |
| 144             | 1.27                  | 2.44                    | 3.11                | -3.05  | -0.81 | 1.97  |
| 168             | 1.17                  | 2.42                    | 3.06                | -10.69 | -1.63 | 0.33  |
| 192             | 1.14                  | 2.43                    | 3.11                | -12.98 | -1.22 | 1.97  |
| 216             | 1.15                  | 2.51                    | 3.18                | -12.21 | 2.03  | 4.26  |
| 240             | 1.11                  | 2.42                    | 3.04                | -15.27 | -1.63 | -0.33 |
| 312             | 1.15                  | 2.58                    | 3.24                | -12.21 | 4.88  | 6.23  |

The results show that the stability of the color developer solution is similar to that of Comparative Example 4.

#### COMPARATIVE EXAMPLE 6

This example was used to demonstrate the temperature dependence of the Dmin increase of the conventional C-41 color developer solution when it is "aged" for extended periods of time at 50° C. Processing was conducted as described in Comparative Example 2. The results are shown in Tables XV and XVI.

TABLE XV

| Time<br>(Hours) | Dmin<br>Red<br>Record | Dmin<br>Green<br>Record | Dmin Blue<br>Record | % Cr  | % Cg | % Cb |
|-----------------|-----------------------|-------------------------|---------------------|-------|------|------|
| 0               | 0.260                 | 0.672                   | 0.951               | 0.00  | 0.00 | 0.00 |
| 24              | 0.253                 | 0.693                   | 0.954               | -2.69 | 3.12 | 0.32 |
| 96              | 0.266                 | 0.699                   | 0.964               | 2.31  | 4.02 | 1.37 |
| 120             | 0.264                 | 0.685                   | 0.965               | 1.54  | 1.93 | 1.47 |
| 144             | 0.261                 | 0.695                   | 0.974               | 0.38  | 3.42 | 2.42 |
| 264             | 0.274                 | 0.699                   | 0.988               | 5.38  | 4.02 | 3.89 |
| 336             | 0.277                 | 0.711                   | 1.014               | 6.54  | 5.80 | 6.62 |
| 432             | 0.285                 | 0.713                   | 1.040               | 9.62  | 6.10 | 9.36 |

TABLE XVI

| Time<br>(Hours) | Dmax<br>Red<br>Record | Dmax<br>Green<br>Record | Dmax Blue<br>Record | % Cr  | % Cg | % Cb |
|-----------------|-----------------------|-------------------------|---------------------|-------|------|------|
| 0               | 1.04                  | 2.05                    | 2.58                | 0.00  | 0.00 | 0.00 |
| 24              | 1.02                  | 2.07                    | 2.60                | -1.92 | 0.98 | 0.78 |

TABLE XVI-continued

| Time<br>(Hours) | Dmax Red<br>Record | Dmax<br>Green<br>Record | Dmax<br>Blue<br>Record | % Cr | % Cg | % Cb |
|-----------------|--------------------|-------------------------|------------------------|------|------|------|
| 96              | 1.13               | 2.16                    | 2.71                   | 8.65 | 5.37 | 5.04 |
| 120             | 1.12               | 2.13                    | 2.68                   | 7.69 | 3.90 | 3.88 |
| 144             | 1.12               | 2.14                    | 2.71                   | 7.69 | 4.39 | 5.04 |
| 264             | 1.14               | 2.16                    | 2.70                   | 9.62 | 5.37 | 4.65 |
| 336             | 1.12               | 2.09                    | 2.65                   | 7.69 | 1.95 | 2.71 |
| 432             | 1.06               | 2.07                    | 2.63                   | 1.92 | 0.98 | 1.94 |

The data in Table XV show that the higher processing temperature produced undesirable Dmin increases in all color records. The changes are not as large as when the processing was at 57.5° C., but they are still too significant and are present in all color records. The changes in the Dmax for all color records are of the same magnitude as those observed in the standard C-41 process.

20

#### INVENTION EXAMPLE 3

In this example, N-isopropyl-N-(2-ethanesulfonic acid) hydroxylamine (0.026 mol/l) was used as the antioxidant in the color developer solution. It was aged at 50° C., and processing was like Comparative Example 2. The density changes in the color records are shown in Tables XVII and XVIII below.

30

TABLE XVII

| Time<br>(Hours) | Dmin Red<br>Record | Dmin<br>Green<br>Record | Dmin Blue<br>Record | % Cr  | % Cg | % Cb |
|-----------------|--------------------|-------------------------|---------------------|-------|------|------|
| 0               | 0.277              | 0.698                   | 0.966               | 0.00  | 0.00 | 0.00 |
| 24              | 0.273              | 0.721                   | 0.973               | -1.44 | 3.30 | 0.72 |
| 96              | 0.271              | 0.707                   | 0.974               | -2.17 | 1.29 | 0.83 |
| 120             | 0.274              | 0.717                   | 0.975               | -1.08 | 2.72 | 0.93 |
| 144             | 0.278              | 0.727                   | 0.984               | 0.36  | 4.15 | 1.86 |
| 264             | 0.281              | 0.715                   | 0.987               | 1.44  | 2.44 | 2.17 |
| 336             | 0.284              | 0.727                   | 0.990               | 2.53  | 4.15 | 2.48 |
| 432             | 0.287              | 0.714                   | 0.993               | 3.61  | 2.29 | 2.80 |

45

TABLE XVIII

| Time<br>(Hours) | Dmax Red<br>Record | Dmax<br>Green<br>Record | Dmax<br>Blue<br>Record | % Cr  | % Cg  | % Cb  |
|-----------------|--------------------|-------------------------|------------------------|-------|-------|-------|
| 0               | 1.30               | 2.37                    | 2.95                   | 0.00  | 0.00  | 0.00  |
| 24              | 1.23               | 2.32                    | 2.85                   | -5.38 | -2.11 | -3.39 |
| 96              | 1.24               | 2.28                    | 2.86                   | -4.62 | -3.80 | -3.05 |
| 120             | 1.26               | 2.32                    | 2.89                   | -3.08 | -2.11 | -2.03 |
| 144             | 1.28               | 2.34                    | 2.90                   | -1.54 | -1.27 | -1.69 |
| 264             | 1.31               | 2.35                    | 3.00                   | 0.77  | -0.84 | 0.00  |
| 336             | 1.34               | 2.39                    | 2.96                   | 3.08  | 0.84  | 0.34  |
| 432             | 1.32               | 2.51                    | 3.14                   | 1.54  | 5.91  | 6.44  |

55

The results in Table XVII show that the changes in Dmin as a function of time are much improved relative to Comparative Example 6. The small changes in Dmax, as shown in Table XVIII, demonstrate the stability of the color developer solution.

60

#### COMPARATIVE EXAMPLE 7

In this experiment, conventional N,N-diethylhydroxylamine (0.029 mol/l) was used as the antioxidant in the color developer solution, and the sodium bromide concentration was increased to 0.051 mol/l. Aging

65

## 19

and processing were conducted as described in Comparative Example 2. The density changes in the color records are shown in Tables XIX and XX below.

TABLE XIX

| Time<br>(Hours) | Dmin Red<br>Record | Dmin<br>Green<br>Record | Dmin Blue<br>Record | % Cr  | % Cg  | % Cb |
|-----------------|--------------------|-------------------------|---------------------|-------|-------|------|
| 0               | 0.255              | 0.668                   | 0.953               | 0.00  | 0.00  | 0.00 |
| 72              | 0.330              | 0.776                   | 1.023               | 29.41 | 16.17 | 7.35 |
| 120             | 0.318              | 0.757                   | 1.022               | 24.71 | 13.32 | 7.24 |
| 264             | 0.306              | 0.737                   | 1.028               | 20.00 | 10.33 | 7.87 |
| 408             | 0.281              | 0.714                   | 1.015               | 10.20 | 6.89  | 6.51 |

TABLE XX

| Time<br>(Hours) | Dmax Red<br>Record | Dmax<br>Green<br>Record | Dmax<br>Blue<br>Record | % Cr  | % Cg  | % Cb  |
|-----------------|--------------------|-------------------------|------------------------|-------|-------|-------|
| 0               | 1.16               | 2.11                    | 2.70                   | 0.00  | 0.00  | 0.00  |
| 72              | 1.41               | 2.43                    | 3.15                   | 21.55 | 15.17 | 16.67 |
| 120             | 1.36               | 2.35                    | 3.04                   | 17.24 | 11.37 | 12.59 |
| 264             | 1.26               | 2.29                    | 2.99                   | 8.62  | 8.53  | 10.74 |
| 408             | 1.07               | 2.22                    | 2.92                   | -7.76 | 5.21  | 8.15  |

The results show an unacceptable Dmin increase in the three color records after three days of "aging" of the color developer. The Dmin increases decreases thereafter, but remains unacceptably high. The Dmax changes in the same manner as the Dmin.

The invention has been described in detail with particular reference to preferred embodiments thereof, but it will be understood that variations and modifications can be effected within the spirit and scope of the invention.

I claim:

1. A method of photoprocessing comprising:
  - A) color developing an imagewise exposed color negative photographic film element containing at least one silver bromoiodide emulsion, with a color developer solution that comprises:
    - a color developing agent present at from about 0.01 to about 0.1 mol/l, and
    - an antioxidant present at from about 0.001 to about 0.5 mol/l, said antioxidant having the formula:



wherein L and L' are independently alkylene of 1 to 8 carbon atoms or alkylenephenylene of 1 to 3 carbon atoms in the alkylene portion, and R and R' are independently hydrogen, carboxy, sulfo or phosphono, provided that at least one of R and R' is not hydrogen,

said contacting being carried out at from about 45° to about 65° C. for from about 20 to about 150 seconds, provided that said photographic film element exhibits a ΔDmin of less than 10% when processed with said color developer solution that has been held at 57.5° C. for up to 320 hours prior to processing, wherein ΔDmin is defined as:

$$\Delta D_{min} = (1\% Cr + 1\% Cg + 1\% Cb)/3$$

$$\% C_i = \left[ \frac{D_{min,i}(t) - D_{min,i}(0)}{D_{min,i}(0)} \right] \times 100$$

"i" is r (red), g (green), or b (blue), and "t" is time.

## 20

2. The method of claim 1 wherein said silver bromoiodide emulsion comprises from about 0.05 to about 10 mol % iodide based on total silver.

3. The method of claim 1 wherein said photographic film element comprises at least two separate light sensitive emulsion layers, and each layer comprises a silver bromoiodide emulsion.

4. The method of claim 1 wherein said contacting is carried out at from about 50° to about 65° C. for from about 30 to about 120 seconds.

5. The method of claim 4 wherein said contacting is carried out at from about 55° to about 60° C. for from about 30 to about 90 seconds.

15 6. The method of claim 1 wherein said antioxidant is present in an amount of from about 0.005 to about 0.5 mol/l.

7. The method of claim 1 wherein L and L' are independently alkylene of 3 to 6 carbon atoms, or alkylenephenylene having 1 or 2 carbon atoms in the alkylene portion.

8. The method of claim 1 wherein L and L' are the same.

9. The method of claim 8 wherein L and L' are independently alkylene of 3 to 6 carbon atoms that are branched at the carbon atom directly attached to the nitrogen atom.

20 10. The method of claim 8 wherein L is alkylene branched at the carbon atom directly attached to the nitrogen atom, and L' is a linear alkylene.

11. The method of claim 1 wherein R and R' are independently hydrogen, carboxy or sulfo.

12. The method of claim 1 wherein R and R' are independently hydrogen or sulfo.

13. The method of claim 1 wherein said antioxidant is N-isopropyl-N-(2-ethanesulfonic acid)hydroxylamine, N,N-bis(propionic acid)hydroxylamine, N,N-bis(2-ethanesulfonic acid)hydroxylamine, N-isopropyl-N-(n-propylsulfonic acid)hydroxylamine, N-2-ethanephosphonic acid-N-(propionic acid)hydroxylamine, N,N-bis(2-ethanephosphonic acid)hydroxylamine, N-sec-butyl-N-(2-ethanesulfonic acid)hydroxylamine, N,N-bis(sec-butylcarboxylic acid)hydroxylamine, N-methyl-N-(p-carboxylbenzyl)hydroxylamine, N-isopropyl-N-(p-carboxylbenzyl)hydroxylamine, N,N-bis(p-carboxylbenzyl)hydroxylamine, N-methyl-N-(p-carboxyl-m-methylbenzyl)hydroxylamine, N-isopropyl-N-(p-sulfonylbenzyl)hydroxylamine, N-ethyl-N-(p-phosphonobenzyl)hydroxylamine, N-isopropyl-N-(2-carboxymethylene-3-propionic acid)hydroxylamine, or an alkali metal salt thereof.

35 45 50 55 60 65 70 75 80 85 90 95 100 105 110 115 120 125 130 135 140 145 150 155 160 165 170 175 180 185 190 195 200 205 210 215 220 225 230 235 240 245 250 255 260 265 270 275 280 285 290 295 300 305 310 315 320 325 330 335 340 345 350 355 360 365 370 375 380 385 390 395 400 405 410 415 420 425 430 435 440 445 450 455 460 465 470 475 480 485 490 495 500 505 510 515 520 525 530 535 540 545 550 555 560 565 570 575 580 585 590 595 600 605 610 615 620 625 630 635 640 645 650 655 660 665 670 675 680 685 690 695 700 705 710 715 720 725 730 735 740 745 750 755 760 765 770 775 780 785 790 795 800 805 810 815 820 825 830 835 840 845 850 855 860 865 870 875 880 885 890 895 900 905 910 915 920 925 930 935 940 945 950 955 960 965 970 975 980 985 990 995 1000 1005 1010 1015 1020 1025 1030 1035 1040 1045 1050 1055 1060 1065 1070 1075 1080 1085 1090 1095 1100 1105 1110 1115 1120 1125 1130 1135 1140 1145 1150 1155 1160 1165 1170 1175 1180 1185 1190 1195 1200 1205 1210 1215 1220 1225 1230 1235 1240 1245 1250 1255 1260 1265 1270 1275 1280 1285 1290 1295 1300 1305 1310 1315 1320 1325 1330 1335 1340 1345 1350 1355 1360 1365 1370 1375 1380 1385 1390 1395 1400 1405 1410 1415 1420 1425 1430 1435 1440 1445 1450 1455 1460 1465 1470 1475 1480 1485 1490 1495 1500 1505 1510 1515 1520 1525 1530 1535 1540 1545 1550 1555 1560 1565 1570 1575 1580 1585 1590 1595 1600 1605 1610 1615 1620 1625 1630 1635 1640 1645 1650 1655 1660 1665 1670 1675 1680 1685 1690 1695 1700 1705 1710 1715 1720 1725 1730 1735 1740 1745 1750 1755 1760 1765 1770 1775 1780 1785 1790 1795 1800 1805 1810 1815 1820 1825 1830 1835 1840 1845 1850 1855 1860 1865 1870 1875 1880 1885 1890 1895 1900 1905 1910 1915 1920 1925 1930 1935 1940 1945 1950 1955 1960 1965 1970 1975 1980 1985 1990 1995 2000 2005 2010 2015 2020 2025 2030 2035 2040 2045 2050 2055 2060 2065 2070 2075 2080 2085 2090 2095 2100 2105 2110 2115 2120 2125 2130 2135 2140 2145 2150 2155 2160 2165 2170 2175 2180 2185 2190 2195 2200 2205 2210 2215 2220 2225 2230 2235 2240 2245 2250 2255 2260 2265 2270 2275 2280 2285 2290 2295 2300 2305 2310 2315 2320 2325 2330 2335 2340 2345 2350 2355 2360 2365 2370 2375 2380 2385 2390 2395 2400 2405 2410 2415 2420 2425 2430 2435 2440 2445 2450 2455 2460 2465 2470 2475 2480 2485 2490 2495 2500 2505 2510 2515 2520 2525 2530 2535 2540 2545 2550 2555 2560 2565 2570 2575 2580 2585 2590 2595 2600 2605 2610 2615 2620 2625 2630 2635 2640 2645 2650 2655 2660 2665 2670 2675 2680 2685 2690 2695 2700 2705 2710 2715 2720 2725 2730 2735 2740 2745 2750 2755 2760 2765 2770 2775 2780 2785 2790 2795 2800 2805 2810 2815 2820 2825 2830 2835 2840 2845 2850 2855 2860 2865 2870 2875 2880 2885 2890 2895 2900 2905 2910 2915 2920 2925 2930 2935 2940 2945 2950 2955 2960 2965 2970 2975 2980 2985 2990 2995 3000 3005 3010 3015 3020 3025 3030 3035 3040 3045 3050 3055 3060 3065 3070 3075 3080 3085 3090 3095 3100 3105 3110 3115 3120 3125 3130 3135 3140 3145 3150 3155 3160 3165 3170 3175 3180 3185 3190 3195 3200 3205 3210 3215 3220 3225 3230 3235 3240 3245 3250 3255 3260 3265 3270 3275 3280 3285 3290 3295 3300 3305 3310 3315 3320 3325 3330 3335 3340 3345 3350 3355 3360 3365 3370 3375 3380 3385 3390 3395 3400 3405 3410 3415 3420 3425 3430 3435 3440 3445 3450 3455 3460 3465 3470 3475 3480 3485 3490 3495 3500 3505 3510 3515 3520 3525 3530 3535 3540 3545 3550 3555 3560 3565 3570 3575 3580 3585 3590 3595 3600 3605 3610 3615 3620 3625 3630 3635 3640 3645 3650 3655 3660 3665 3670 3675 3680 3685 3690 3695 3700 3705 3710 3715 3720 3725 3730 3735 3740 3745 3750 3755 3760 3765 3770 3775 3780 3785 3790 3795 3800 3805 3810 3815 3820 3825 3830 3835 3840 3845 3850 3855 3860 3865 3870 3875 3880 3885 3890 3895 3900 3905 3910 3915 3920 3925 3930 3935 3940 3945 3950 3955 3960 3965 3970 3975 3980 3985 3990 3995 4000 4005 4010 4015 4020 4025 4030 4035 4040 4045 4050 4055 4060 4065 4070 4075 4080 4085 4090 4095 4100 4105 4110 4115 4120 4125 4130 4135 4140 4145 4150 4155 4160 4165 4170 4175 4180 4185 4190 4195 4200 4205 4210 4215 4220 4225 4230 4235 4240 4245 4250 4255 4260 4265 4270 4275 4280 4285 4290 4295 4300 4305 4310 4315 4320 4325 4330 4335 4340 4345 4350 4355 4360 4365 4370 4375 4380 4385 4390 4395 4400 4405 4410 4415 4420 4425 4430 4435 4440 4445 4450 4455 4460 4465 4470 4475 4480 4485 4490 4495 4500 4505 4510 4515 4520 4525 4530 4535 4540 4545 4550 4555 4560 4565 4570 4575 4580 4585 4590 4595 4600 4605 4610 4615 4620 4625 4630 4635 4640 4645 4650 4655 4660 4665 4670 4675 4680 4685 4690 4695 4700 4705 4710 4715 4720 4725 4730 4735 4740 4745 4750 4755 4760 4765 4770 4775 4780 4785 4790 4795 4800 4805 4810 4815 4820 4825 4830 4835 4840 4845 4850 4855 4860 4865 4870 4875 4880 4885 4890 4895 4900 4905 4910 4915 4920 4925 4930 4935 4940 4945 4950 4955 4960 4965 4970 4975 4980 4985 4990 4995 5000 5005 5010 5015 5020 5025 5030 5035 5040 5045 5050 5055 5060 5065 5070 5075 5080 5085 5090 5095 5100 5105 5110 5115 5120 5125 5130 5135 5140 5145 5150 5155 5160 5165 5170 5175 5180 5185 5190 5195 5200 5205 5210 5215 5220 5225 5230 5235 5240 5245 5250 5255 5260 5265 5270 5275 5280 5285 5290 5295 5300 5305 5310 5315 5320 5325 5330 5335 5340 5345 5350 5355 5360 5365 5370 5375 5380 5385 5390 5395 5400 5405 5410 5415 5420 5425 5430 5435 5440 5445 5450 5455 5460 5465 5470 5475 5480 5485 5490 5495 5500 5505 5510 5515 5520 5525 5530 5535 5540 5545 5550 5555 5560 5565 5570 5575 5580 5585 5590 5595 5600 5605 5610 5615 5620 5625 5630 5635 5640 5645 5650 5655 5660 5665 5670 5675 5680 5685 5690 5695 5700 5705 5710 5715 5720 5725 5730 5735 5740 5745 5750 5755 5760 5765 5770 5775 5780 5785 5790 5795 5800 5805 5810 5815 5820 5825 5830 5835 5840 5845 5850 5855 5860 5865 5870 5875 5880 5885 5890 5895 5900 5905 5910 5915 5920 5925 5930 5935 5940 5945 5950 5955 5960 5965 5970 5975 5980 5985 5990 5995 6000 6005 6010 6015 6020 6025 6030 6035 6040 6045 6050 6055 6060 6065 6070 6075 6080 6085 6090 6095 6100 6105 6110 6115 6120 6125 6130 6135 6140 6145 6150 6155 6160 6165 6170 6175 6180 6185 6190 6195 6200 6205 6210 6215 6220 6225 6230 6235 6240 6245 6250 6255 6260 6265 6270 6275 6280 6285 6290 6295 6300 6305 6310 6315 6320 6325 6330 6335 6340 6345 6350 6355 6360 6365 6370 6375 6380 6385 6390 6395 6400 6405 6410 6415 6420 6425 6430 6435 6440 6445 6450 6455 6460 6465 6470 6475 6480 6485 6490 6495 6500 6505 6510 6515 6520 6525 6530 6535 6540 6545 6550 6555 6560 6565 6570 6575 6580 6585 6590 6595 6600 6605 6610 6615 6620 6625 6630 6635 6640 6645 6650 6655 6660 6665 6670 6675 6680 6685 6690 6695 6700 6705 6710 6715 6720 6725 6730 6735 6740 6745 6750 6755 6760 6765 6770 6775 6780 6785 6790 6795 6800 6805 6810 6815 6820 6825 6830 6835 6840 6845 6850 6855 6860 6865 6870 6875 6880 6885 6890 6895 6900 6905 6910 6915 6920 6925 6930 6935 6940 6945 6950 6955 6960 6965 6970 6975 6980 6985 6990 6995 7000 7005 7010 7015 7020 7025 7030 7035 7040 7045 7050 7055 7060 7065 7070 7075 7080 7085 7090 7095 7100 7105 7110 7115 7120 7125 7130 7135 7140 7145 7150 7155 7160 7165 7170 7175 7180 7185 7190 7195 7200 7205 7210 7215 7220 7225 7230 7235 7240 7245 7250 7255 7260 7265 7270 7275 7280 7285 7290 7295 7300 7305 7310 7315 7320 7325 7330 7335 7340 7345 7350 7355 7360 7365 7370 7375 7380 7385 7390 7395 7400 7405 7410 7415 7420 7425 7430 7435 7440 7445 7450 7455 7460 7465 7470 7475 7480 7485 7490 7495 7500 7505 7510 7515 7520 7525 7530 7535 7540 7545 7550 7555 7560 7565 7570 7575 7580 7585 7590 7595 7600 7605 7610 7615 7620 7625 7630 7635 7640 7645 7650 7655 7660 7665 7670 7675 7680 7685 7690 7695 7700 7705 7710 7715 7720 7725 7730 7735 7740 7745 7750 7755 7760 7765 7770 7775 7780 7785 7790 7795 7800 7805 7810 7815 7820 7825 7830 7835 7840 7845 7850 7855 7860 7865 7870 7875 7880 7885 7890 7895 7900 7905 7910 7915 7920 7925 7930 7935 7940 7945 7950 7955 7960 7965 7970 7975 7980 7985 7990 7995 8000 8005 8010 8015 8020 8025 8030 8035 8040 804

**21**

with a color developer solution comprising:  
 a color developing agent present at from about 0.01 to  
 about 0.1 mol/l, and  
 an antioxidant present at from about 0.001 to about 0.5  
 mol/l, said antioxidant having the formula:



wherein L and L' are independently alkylene of 3 to 5 carbon atoms, at least one of L and L' being an alkylene that is branched at the carbon atom attached to the nitrogen atom, and R and R' are independently hydrogen, carboxy or sulfo, provided that at least one of R and R' is not hydrogen,

said color developing being carried out at from about 50° to about 60° C. for from about 30 to about 90 seconds,

5

10

**22**

provided that said photographic film element exhibits a ΔD<sub>min</sub> of less than 10% when processed with said color developer solution that has been held at 57.5° C. for up to 320 hours prior to processing,  
 B) bleaching said color developed element,  
 C) fixing said bleached element, and  
 D) washing or rinsing said fixed element.

**18.** The method of claim 17 wherein said color developer solution has a pH of from about 10 to about 11, and comprises bromide ions in a concentration of from about  $5 \times 10^{-5}$  to about 0.4 mol/l, and iodide ions in a concentration of from about  $5 \times 10^{-7}$  to about 0.01 mol/l.

\* \* \* \* \*